

## UNITED STATES PATENT OFFICE.

JOSEPH GALLIAN, OF SAN FRANCISCO, CALIFORNIA.

## WATERPROOF PAINT.

No Drawing.

Application filed December 13, 1924. Serial No. 755,719.

To all whom it may concern:

Be it known that I, JOSEPH GALLIAN, a citizen of the United States, residing at San Francisco, in the county of San Francisco and State of California, have invented new and useful Improvements in Waterproof Paint, of which the following is a specification.

The object of the present invention is to provide an improved water-proof paint especially advantageous for facing outside cement walls and bricks.

In practicing my invention, I mix one half of a gallon of a thinner preferably turpentine, one half of a pound of a gum, preferably damar gum to give coherency, one and one half of a pound of wax, preferably beeswax, and one-half ounce of saltpeter to neutralize the dampness in the cement of the structure. These are cooked for fifteen minutes in a kettle having a water jacket containing water at a boiling temperature. I then add to the cooked mixture three-eighths of a gallon of white lead, preferably what is known as "combination

white lead". This is a mixture of the following ingredients:

|                 | Pounds. |
|-----------------|---------|
| Zinc oxide      | 3.61    |
| Lead carbonate  | 3.61    |
| Barium sulphate | 3.61    |
| Linseed oil     | 1.17    |

This makes twelve pounds in all. These ingredients are mixed and ground together. Then after thoroughly mixing the combination lead with the other ingredients, I cook the same in the water jacketed kettle for ten minutes. I thus obtain one gallon of my improved paint, which is now ready for use and should be applied while still hot in order that all the ingredients may be well mixed. The material is especially effective as a water-proof facing for outside concrete walls and bricks.

I claim:

A composition of matter comprising a combination of white lead, turpentine, damar gum, beeswax, and saltpeter, substantially in the proportions specified.

JOSEPH GALLIAN.